

# UNITED STATES PATENT OFFICE.

JAMES FOLEY, OF MONTREAL, QUEBEC, CANADA.

## TANNING COMPOUND.

SPECIFICATION forming part of Letters Patent No. 237,007, dated January 25, 1881.

Application filed November 3, 1880. (No specimens.)

*To all whom it may concern:*

Be it known that I, JAMES FOLEY, of the city of Montreal, in the Province of Quebec, Canada, have invented certain new and useful 5 Improvements in Aqueous Solutions of Tannin or Tanning-Ooze; and I do hereby declare the following to be a full and complete description of the same.

This invention has reference to the preservation and protection of tannin or tannic acid from the deteriorations to which it is subject in aqueous solutions and in tanning extracts prepared from bark and other tanning materials, and to the modification of the red coloring-matters in tanning-ooze; and the object of my said invention is to preserve and protect the tannic acid in tanning solutions or ooze and in semi-liquid tanning extracts from decomposition and conversion into gallic acid, to 20 modify the red coloring-matter in tanning solutions or ooze and its effect upon the tanned leather.

The various kinds of bark and tanning materials yield (apart from the tannic acid) a variety of soluble extractive matters which exist in the ooze with the tannic acid. These extractive matters are capable of inducing fermentation in the solution or ooze, the decomposition of the tannic acid, and its conversion 30 into gallic acid, which is not absorbed by the hides or skins, thus causing a material loss to the tanner. These extractive matters also produce a red coloring-matter in the tanning-ooze, which becomes permanently attached to the hide while being tanned, and gives an objectionable red color to the finished leather and to its grain when buffed, which depreciates its value. This coloring-matter seems to be generated through a kind of fermentation in the 40 tanning-ooze, which comes on suddenly both in cold and warm weather, but more particularly in the latter.

Through extensive practical experiments I have found that by the incorporation of a concentrated liquor or extract, varying in density from 10° to 60° Twaddle, obtained from the wood of the *Morus tinctoria*, the decomposition of the tannic acid and its conversion into gallic acid is prevented, the formation of the red 50 coloring-matter checked, and its effect upon the hides in the process of tanning is so modi-

fied that a leather light in color throughout its entire thickness, with a grain of a good oak color, is produced, which will command at least ten to fifteen per cent. higher price than can 55 be obtained for the red leather now made.

I incorporate the concentrated liquor or extract obtained from the wood of the *Morus tinctoria* by adding it to tanning solutions or ooze prepared from all kinds of tanning materials. 60 The quantity will vary according to the varying strengths of the tanning solutions or ooze. I have found the following proportions to be the most effective and economical for general use, viz: To every one hundred gallons of the 65 tanning solution or ooze of from 6° to 15° of strength by what is termed the "barkometer" I add one gallon of the concentrated liquor or extract obtained from the wood of the *Morus tinctoria* if its specific gravity is from 40° to 70 50° Twaddle, and one and one-half gallon if the specific gravity is from 12° to 20° Twaddle; and if the tanning solution or ooze is from 20° to 30° of strength by the barkometer, I add one and one-half gallon of the liquor or extract from the wood of the *Morus tinctoria*, if 75 of 40° to 50° Twaddle, and two gallons if 12° to 20° Twaddle, to every one hundred gallons of the tanning solution or ooze, thoroughly incorporating them together. 80

The concentrated liquor or extract obtained from the wood of the *Morus tinctoria* may be added to or incorporated with semi-liquid tanning extracts in the proportion of twenty pounds, in weight, of the specific gravity of 85 50° to 60° Twaddle, to every one hundred pounds, in weight, of the semi-liquid tanning extract, to preserve it from the hereinbefore-mentioned deteriorations and to modify the coloring-matter therein. The exact proportions 90 are not material to the successful carrying out of my said invention.

Aqueous solutions of tannin or tanning-ooze in which the concentrated liquor or extract obtained from the wood of the *Morus tinctoria* 95 is incorporated may be concentrated to a semi-liquid state by any suitable method employed for concentrating fluids.

By the incorporation of the concentrated liquor or extract obtained from the wood of the *Morus tinctoria* with tanning-ooze a large saving is effected in the consumption of tannic 100

acid, and consequently in tanning materials, which is all important to the tanner, and a light-colored leather of superior quality is obtained.

5 What I claim as my invention, and desire to secure by Letters Patent, is—

The compound described, consisting of an ooze or solution containing tannic acid, to which the concentrated liquor or extract of the

wood of the *Morus tinctoria* is incorporated, as 10 and for the purpose set forth.

In testimony that I claim the foregoing I have hereunto set my hand this 29th day of October, 1880.

JAMES FOLEY.

Witnesses:

ELMER J. MORGAN,  
GEO. A. GOODYEAR.